



US012522900B2

(12) **United States Patent**  
**Fujiyoshi et al.**

(10) **Patent No.:** **US 12,522,900 B2**  
(45) **Date of Patent:** **Jan. 13, 2026**

|      |                                                                                                                              |    |              |                                                                                                                                                                                                                                                   |
|------|------------------------------------------------------------------------------------------------------------------------------|----|--------------|---------------------------------------------------------------------------------------------------------------------------------------------------------------------------------------------------------------------------------------------------|
| (54) | <b>FE-CO-BASED ALLOY BAR</b>                                                                                                 | JP | 2002194475   | 7/2002                                                                                                                                                                                                                                            |
|      |                                                                                                                              | JP | 2004515644   | 5/2004                                                                                                                                                                                                                                            |
| (71) | Applicant: <b>Proterial, Ltd.</b> , Tokyo (JP)                                                                               | JP | 2004277842 X | 10/2004                                                                                                                                                                                                                                           |
|      |                                                                                                                              | JP | 2006336038   | 12/2006                                                                                                                                                                                                                                           |
| (72) | Inventors: <b>Masaru Fujiyoshi</b> , Tokyo (JP);<br><b>Shujiroh Uesaka</b> , Tokyo (JP); <b>Kouji Kobayashi</b> , Tokyo (JP) | KR | 20020095108  | 12/2002                                                                                                                                                                                                                                           |
|      |                                                                                                                              | WO | 2019059256   | 3/2019                                                                                                                                                                                                                                            |
|      |                                                                                                                              | WO | 2021182518   | 9/2021                                                                                                                                                                                                                                            |
| (73) | Assignee: <b>Proterial, Ltd.</b> , Tokyo (JP)                                                                                |    |              | <b>OTHER PUBLICATIONS</b>                                                                                                                                                                                                                         |
| (*)  | Notice: Subject to any disclaimer, the term of this patent is extended or adjusted under 35 U.S.C. 154(b) by 156 days.       |    |              | Shihao Li et al., "3D printing of ductile equiatomic Fe-Co alloy for soft magnetic applications", Additive Manufacturing, Sep. 10, 2021, pp. 1-9, vol. 47.                                                                                        |
| (21) | Appl. No.: <b>18/037,075</b>                                                                                                 |    |              | Shihao Li et al., "3D printing of ductile equiatomic Fe-Co alloy for soft magnetic applications", Additive Manufacturing, Nov. 1, 2021, pp. 1-12, vol. 47.                                                                                        |
| (22) | PCT Filed: <b>Sep. 14, 2021</b>                                                                                              |    |              | Mohammad R. Kamali et al., "Reobservations of ferrite recrystallization in a cold-rolled ordered Fe-50Co-10V alloy using the EBSD method", Materials Characterization, Oct. 23, 2019, pp. 1-13, vol. 158.                                         |
| (86) | PCT No.: <b>PCT/JP2021/033819</b><br><br>§ 371 (c)(1),<br>(2) Date: <b>May 15, 2023</b>                                      |    |              | Wu; Lai-Zhi et al., "Microstructures of ultra-fine grained FeCoV alloys processed by ECAP plus cold rolling and their evolutions during tempering", Transactions of Nonferrous Metals Society of China, Apr. 2010, pp. 602-606, vol. 20, Issue 4. |
| (87) | PCT Pub. No.: <b>WO2023/042279</b><br><br>PCT Pub. Date: <b>Mar. 23, 2023</b>                                                |    |              | L.C. Zhang et al., "Deformation-induced grain refinement in body-centered cubic Co-Fe alloys upon room temperature compression", Materials Science and Engineering: A, Aug. 20, 2010, pp. 5796-5800, vol. 527, Issues 21-22.                      |
| (65) | <b>Prior Publication Data</b>                                                                                                |    |              | D.F. Susan et al., "The Effects of Annealing After Equal Channel Angular Extrusion (ECAE) on Mechanical and Magnetic Properties of 49Fe-49Co-2V Alloy", Metallurgical and Materials Transactions A, Jul. 9, 2021, pp. 4090-4099, vol. 52.         |
|      | US 2023/0416881 A1 Dec. 28, 2023                                                                                             |    |              | Brahim Nabi et al., "Effect of long range order on mechanical properties of partially recrystallized Fe49Co-2V alloy", Materials Science and Engineering: A, Jan. 13, 2014, pp. 70-76, vol. 592.                                                  |
| (51) | <b>Int. Cl.</b><br><b>C22C 30/00</b> (2006.01)                                                                               |    |              | "Search Report of Europe Related Application, Application No. 21957462.1", issued on Oct. 8, 2024, p. 1-p. 11.                                                                                                                                    |
| (52) | <b>U.S. Cl.</b><br>CPC ..... <b>C22C 30/00</b> (2013.01); <b>C22C 2202/02</b> (2013.01)                                      |    |              |                                                                                                                                                                                                                                                   |
| (58) | <b>Field of Classification Search</b><br>CPC ..... C22C 38/10<br>See application file for complete search history.           |    |              |                                                                                                                                                                                                                                                   |

(Continued)

|                                                             |                           |
|-------------------------------------------------------------|---------------------------|
| (56)                                                        | <b>References Cited</b>   |
| <b>U.S. PATENT DOCUMENTS</b>                                |                           |
| 5,919,319 A * 7/1999 Couderchon ..... C22C 38/10<br>148/309 |                           |
| 6,153,020 A                                                 | 11/2000 Chen et al.       |
| 7,128,790 B2                                                | 10/2006 Waecckerle et al. |
| 2008/0099106 A1                                             | 5/2008 Pieper et al.      |
| 2009/0184790 A1                                             | 7/2009 Pieper et al.      |
| 2014/0338793 A1                                             | 11/2014 Leary et al.      |
| 2018/0119241 A1                                             | 5/2018 Susan et al.       |

**FOREIGN PATENT DOCUMENTS**

|    |            |         |
|----|------------|---------|
| CN | 1596321    | 3/2005  |
| CN | 102296238  | 12/2011 |
| CN | 103691741  | 4/2014  |
| CN | 104708005  | 6/2015  |
| CN | 108130493  | 6/2018  |
| CN | 115279926  | 11/2022 |
| GB | 896881     | 5/1962  |
| GB | 1415552    | 11/1975 |
| JP | S5224915   | 2/1977  |
| JP | S61130419  | 6/1986  |
| JP | H05195170  | 8/1993  |
| JP | H05279784  | 10/1993 |
| JP | H05304014  | 11/1993 |
| JP | H071166239 | 6/1995  |
| JP | H08300044  | 11/1996 |

*Primary Examiner* — Jophy S. Koshy  
*Assistant Examiner* — Joshua S Carpenter  
(74) *Attorney, Agent, or Firm* — JCIPRNET

**(57) ABSTRACT**

The present invention provides an Fe—Co-based alloy bar which enables excellent magnetic properties to be reliably obtained. In the Fe—Co-based alloy bar, an area ratio of crystal grains having a grain orientation spread (GOS) value of 0.5° or more exceeds 80%, and the difference between an area ratio of crystal grains having a GOS value of 0.5° or more observed in a cross section in a direction perpendicular to an axis of the bar and an area ratio of crystal grains having a GOS value of 0.5° or more observed in a cross section in an axial direction of the bar is within 10%. Preferably, the average crystal grain size number is 6.0 or more and 8.5 or less.

(56)

**References Cited**

**OTHER PUBLICATIONS**

“Search Report of Europe Counterpart Application”, issued on Oct. 8, 2024, p. 1-p. 13.

“Requirement for Restriction of U.S. Appl. No. 17/909,438”, issued on Nov. 14, 2024, pp. 1-9.

“Office Action of China Counterpart Application”, issued on Nov. 23, 2024, with English translation thereof, pp. 1-10.

“Office Action of China Related Application No. 202180075803.1”, issued on Nov. 12, 2024, with English translation thereof, pp. 1-12.

“International Search Report (Form PCT/ISA/210) of PCT/JP2021/009570”, mailed on May 25, 2021, with English translation thereof, pp. 1-6.

“International Search Report (Form PCT/ISA/210) of PCT/JP2021/033818”, mailed on Nov. 30, 2021, with English translation thereof, pp. 1-6.

“International Search Report (Form PCT/ISA/210) of PCT/JP2021/033819”, mailed on Nov. 30, 2021, with English translation thereof, pp. 1-4.

“Office Action of China Related Application No. 202180019418.5”, issued on Mar. 12, 2024, with English translation thereof, p. 1-p. 11.

“Office Action of U.S. Related Application, U.S. Appl. No. 18/037,073”, issued on Feb. 13, 2025, p. 1-p. 29.

Mohamed Sakr et al., “A comprehensive review on applications of ohmic heating (OH)”, Renewable and Sustainable Energy Reviews, Jul. 31, 2014, pp. 262-269, vol. 39.

“Office Action of U.S. Co-Pending Application, U.S. Appl. No. 17/909,438”, issued on Feb. 12, 2025, p. 1-p. 32.

“Office Action of U.S. Appl. No. 17/909,438”, issued on Jul. 16, 2025, pp. 1-26.

“Office Action of U.S. Appl. No. 18/037,073”, issued on Jul. 22, 2025, pp. 1-23.

Martin Raulf, Karin Persson, “Rolling of Steel”, Encyclopedia of Lubricants and Lubrication, Theo Mang (eds), 2014, pp. 1663-1680.

\* cited by examiner

**FE-CO-BASED ALLOY BAR****CROSS-REFERENCE TO RELATED APPLICATION**

This application is a 371 application of the International PCT application serial no. PCT/JP2021/033819, filed on Sep. 14, 2021. The entirety of each of the above-mentioned patent applications is hereby incorporated by reference herein and made a part of this specification.

**TECHNICAL FIELD**

The present invention relates to an Fe—Co-based alloy bar.

**BACKGROUND ART**

Bars of an Fe—Co-based alloy represented by Permendur, which is known as an alloy having excellent magnetic properties, are used in various products such as sensors, cylindrical magnetic shields, solenoid valves, and magnetic cores. As a method for manufacturing an Fe—Co-based alloy bar, for example, Patent Literature 1 describes that an ingot is heated to 1,000° C. to 1,100° C. and then hot-processed into a billet of about 990 mm, scratches on the surface and the like are removed with a lathe, heating is performed at 1,000° C. to 1,100° C., and then a hot-rolled material (bar) of about φ6 to φ9 mm is produced.

**CITATION LIST****Patent Literature**

[Patent Literature 1]

Japanese Patent Laid-Open No. H7-166239

**SUMMARY OF INVENTION****Technical Problem**

Along with higher performance of the above products, further improvement in magnetic properties is also required for materials. Therefore, an objective of the present invention is to provide an Fe—Co-based alloy bar which enables excellent magnetic properties to be reliably obtained.

**Solution to Problem**

The present invention has been made in view of the above circumstances. That is, the present invention provides an Fe—Co-based alloy bar in which an area ratio of crystal grains having a grain orientation spread (GOS) value of 0.5° or more exceeds 80%, and the difference between an area ratio of crystal grains having a GOS value of or more observed in a cross section in a direction perpendicular to an axis of the bar and an area ratio of crystal grains having a GOS value of 0.5° or more observed in a cross section in an axial direction of the bar is within 10%. Preferably, the average crystal grain size number is 6.0 or more and 8.5 or less.

**Advantageous Effects of Invention**

According to the present invention, it is possible to reliably obtain an Fe—Co-based alloy bar having excellent magnetic properties.

**DESCRIPTION OF EMBODIMENTS**

Hereinafter, an embodiment of the present invention will be described. The Fe—Co-based alloy bar of the present invention is a straight bar-shaped bar having a circular (or elliptic) cross-sectional shape or a rectangular cross-sectional shape. When the Fe—Co-based alloy bar is a round bar, the diameter is 5 to 20 mm. Here, regarding bars other than round bars, the equivalent circle diameter of the horizontal cross section may be 5 to 20 mm. Unless otherwise specified, the bar of the present embodiment is a round bar having a circular cross-sectional shape.

**<Hot-Rolled Material Composition>**

First, in the present embodiment, a hot-rolled material of an Fe—Co-based alloy is prepared. The Fe—Co-based alloy in the present invention refers to an alloy material containing 95% or more of Fe+Co in mass % and containing 25 to 60% of Co. Thereby, a high magnetic flux density can be exhibited.

Next, elements that may be contained in the Fe—Co-based alloy of the present invention will be described. In order to improve processability and magnetic properties, the Fe—Co-based alloy of the present invention may contain a total of one, two or more elements of V, Si, Mn, Al, Zr, B, Ni, Ta, Nb, W, Ti, Mo, and Cr in a maximum mass % of 5.0%. In addition, examples of impurity elements that are unavoidably incorporated include C, S, P, and O, and for example, the upper limit of each element is preferably 0.1%.

An Fe—Co-based alloy bar of the present invention contains more than 80% of crystal grains having a grain orientation spread (GOS) value of 0.5° or more in terms of an area ratio. This GOS value can be measured by a conventionally known “electron backscatter diffraction (SEM-EBSD) method,” and can be derived by calculating the orientation difference of points (pixels) constituting crystal grains. The crystal orientation difference obtained from the GOS value is an index indicating the strain imparted to the alloy by processing, and when the bar contains more than 80% of crystal grains having a GOS value of 0.5° or more in terms of an area ratio, the driving force for crystal grain growth is introduced into the bar, and there is an advantage of favorable magnetic properties being reliably obtained. When the area ratio of crystal grains having a GOS value of 0.5° or more is 80% or less, favorable magnetic properties cannot be reliably obtained because the bar has an insufficient driving force for crystal grain growth. In the crystal grains having a GOS value of 0.5° or more, the area ratio is preferably 82% or more, and the area ratio is more preferably 84% or more. The upper limit of the area ratio of crystal grains having a GOS value of 0.5° or more is not particularly limited, and may be, for example, 99%. Here, the crystal grains having a GOS value of 0.5° or more can be observed in the cross section in the direction perpendicular to the axis of the bar. In addition, the cross section in which the area ratio is observed includes a cross section in the direction perpendicular to the axis and a cross section in the axial direction, but the area ratio is preferably more than 80% (more preferably 82% or more, and still more preferably 84% or more) in both cases of observing the cross section in the direction perpendicular to the axis and the cross section in the axial direction of the bar. This is because the effect of strain due to rolling traces generated in the base material during the hot rolling step is easily observed in the cross section in the axial direction of the bar, and the area ratio observed in the cross section in the axial direction may be smaller than the area ratio observed in the cross section in the direction perpendicular to the axis.

50 Here, the crystal grains having a GOS value of 0.5° or more can be observed in the cross section in the direction perpendicular to the axis of the bar. In addition, the cross section in which the area ratio is observed includes a cross section in the direction perpendicular to the axis and a cross section in the axial direction, but the area ratio is preferably more than 80% (more preferably 82% or more, and still more preferably 84% or more) in both cases of observing the cross section in the direction perpendicular to the axis and the cross section in the axial direction of the bar. This is because the effect of strain due to rolling traces generated in the base material during the hot rolling step is easily observed in the cross section in the axial direction of the bar, and the area ratio observed in the cross section in the axial direction may be smaller than the area ratio observed in the cross section in the direction perpendicular to the axis.

Therefore, even in the cross section in the axial direction in which the area ratio tends to be small, the effect of the present invention can be more reliably achieved if the numerical value of the area ratio is satisfied.

In the Fe—Co-based alloy bar of the present invention, the difference between the area ratio of crystal grains having a GOS value of 0.5° or more observed in the cross section in the direction perpendicular to the axis of the bar and the area ratio of crystal grains having a GOS value of 0.5° or more observed in the cross section in the axial direction of the bar is within 10%. This suggests that, as the difference (anisotropy) between the area ratio observed in the cross section in the direction perpendicular to the axis and the area ratio observed in the cross section in the axial direction becomes larger, the variation in the strain distribution becomes larger, and variation occurs in the crystal grain size of the annealed sample that imparts magnetic properties, which considerably acts to minimize growth of crystal grains, and causes magnetic properties to deteriorate. The difference between the area ratio is preferably within 7%, more preferably within 5%, and still more preferably within 3%.

In addition, the average crystal grain size number of the Fe—Co-based alloy bar of the present invention is preferably 6.0 or more and 8.5 or less. Thereby, superior magnetic properties after magnetic annealing are easily exhibited, and the processability tends to be further improved. The lower limit of the average crystal grain size number is more preferably 6.5 or more, and the upper limit of the average crystal grain size number is more preferably 8.0 or less. Here, the average crystal grain size number can be measured based on JIS G 0551. Thus, it can be measured in the cross section in the direction perpendicular to the axis or the cross section in the axial direction of the bar.

Next, an example of a manufacturing method through which an Fe—Co-based alloy bar of the present invention can be obtained will be described. In the present embodiment, as an intermediate material of the Fe—Co-based alloy bar, a billet obtained from an Fe—Co-based alloy steel ingot having the above components is hot-rolled, and thereby a hot-rolled material can be obtained. Since an oxidized layer is formed by hot rolling in this intermediate material, for example, a polishing step in which the oxidized layer is mechanically or chemically removed may be introduced.

This hot-rolled material has, for example, a shape of a “hot-rolled bar” corresponding to an Fe—Co-based alloy bar. Thus, in consideration of processability in the post-step, the diameter may be 5 to 20 mm. Here, regarding bars other than round bars, the equivalent circle diameter of the horizontal cross section may be 5 to 20 mm.

#### <Solution Treatment Step>

In the present embodiment, a hot-rolled material before a heating straightening step to be described below may be subjected to at least one solution treatment. When this solution treatment is performed, effects of removing component segregation of the hot-rolled material, improving magnetic properties, and improving processability can be expected. If the heating temperature during the solution treatment is too low, the processability tends to deteriorate, and if the heating temperature is too high, deterioration of magnetic properties is caused, and thus it is preferable to

perform the treatment at a temperature of 800 to 1,050° C. The lower limit of the temperature is more preferably 850° C. The upper limit of the temperature is more preferably 950° C., and the upper limit of the temperature is still more preferably 900° C. In addition, the heating time can be set to 10 minutes to 60 minutes. In addition, in the solution treatment step, in order to solid-solutionize harmful precipitates without precipitating them, minimize regularization, and improve processability, a rapid cooling treatment is performed after heating.

#### <Heating Straightening Step>

In the present embodiment, a heating straightening step is performed in which tensile stress is imparted to the above hot-rolled material while heating is performed. In this case, if the hot-rolled material has a “bar” shape, it is pulled in the length direction of the hot-rolled bar, and thus the tensile stress is imparted. According to this step, it is possible to obtain a bar having very favorable magnetic properties and straightness while imparting residual strain to the hot-rolled material. The heating temperature in this case is set to 500 to 900° C. If the temperature is lower than 500° C., the processability decreases, and the bar may break when tensile stress is imparted. On the other hand, if the heating temperature exceeds 900° C., it is not possible to impart a preferable residual strain to the hot-rolled material. In the heating straightening step, the lower limit of the heating temperature is preferably 600° C., and more preferably 700° C. In addition, the upper limit of the heating temperature is preferably 850° C., more preferably 830° C., and still more preferably 800° C. Here, when the above solution treatment step is omitted, the lower limit of the heating temperature is preferably 700° C., more preferably 730° C., and still more preferably 740° C.

In this heating straightening step, it is possible to use a heating means such as ohmic heating in which a direct current flows through a conductive object to be heated and heating is performed with Joule's heat due to the internal resistance of the object to be heated or induction heating, but ohmic heating is preferably applied so that an effect of facilitating aligning of the axis of easy magnetization of crystal grains in the hot-rolled material in a certain direction is obtained and it has an advantage of being able to rapidly (for example, within 1 minute) and uniformly heat the material to a target temperature. In addition, the tension during the heating straightening step is preferably adjusted to 1 to 4 MPa in order to obtain a desired residual strain more reliably. In addition, it is preferable to adjust the elongation to 3 to 10% with respect to the full length before the heating straightening step.

In the present embodiment, regarding the bar that has been subjected to the heating straightening step, centerless polishing may be performed using, for example, a centerless grinder. Thereby, the unfinished surface on the bar surface layer can be removed, and the roundness and tolerance accuracy of the shape can be further improved. In the present invention, since the straightness of the bar is improved according to the heating straightening step, centerless polishing can be performed without cutting a long bar having a length of 1,000 mm or more.

## EXAMPLES

## Example 1

An Fe—Co-based alloy steel ingot having a composition shown in Table 1 was formed into an ingot and then hot-rolled to prepare a  $\Phi 11.5$  mm hot-rolled bar.

<Sample No. 1>

The above hot-rolled bars were subjected to a solution treatment in which the bar was heated at  $850^\circ$  C. and then rapidly cooled, and then subjected to a heating straightening step in which the hot-rolled bar was pulled in the length direction under a condition of a tension of 2.7 MPa while heating so that the temperature of the bar was  $750^\circ$  C. to produce an Fe—Co-based alloy bar of Sample No. 1, which is an example of the present invention.

<Sample No. 2>

The above hot-rolled bar was not subjected to a solution treatment, but a heating straightening step was performed to produce an Fe—Co-based alloy bar of Sample No. 2 which is a comparative example. The conditions for the heating straightening step were the same as those in Sample No. 1.

TABLE 1

| Sample No. | (mass %) |      |      |       |      |                               |
|------------|----------|------|------|-------|------|-------------------------------|
|            | C        | Si   | Mn   | Co    | V    | Remainder                     |
| 1          | 0.01     | 0.04 | 0.13 | 49.01 | 1.97 | Fe and unavoidable impurities |
| 2          | 0.01     | 0.04 | 0.13 | 49.07 | 1.97 | Fe and unavoidable impurities |

Next, the average crystal grain size, the GOS value and the DC magnetic properties of the samples of examples of the present invention and the comparative example were confirmed. For the average crystal grain size, in the horizontal cross section (cross section in the direction perpendicular to the axis), using an optical microscope (commercially available from Olympus), 10 fields of view of  $500 \mu\text{m} \times 350 \mu\text{m}$  were observed, and the particle size number was determined on the crystal grain size standard drawing plate I according to JIS G 0551. The GOS value was determined using a field emission scanning electron microscope (commercially available from ZEISS) and an EBSD measurement/analysis system orientation-imaging-micrograph (OIM) (commercially available from TSL), and the horizontal cross section (cross section in the direction perpendicular to the axis) and the vertical cross section (cross section in the axial direction that passes through the central axis) of the sample were observed. The measurement field of view was  $100 \mu\text{m} \times 100 \mu\text{m}$ , and the step distance between adjacent pixels was  $0.2 \mu\text{m}$ . In addition, observation was performed under the condition in which a boundary having an orientation difference between adjacent pixels of  $5^\circ$  or more was able to be distinguished from a crystal grain boundary, and from the obtained GOS value map, an area ratio with respect to the entire observation field occupied by crystal grains having a GOS value of  $0.5^\circ$  or more was obtained. Regarding the DC magnetic properties, a sample was collected from the obtained bar, and magnetic annealing was then performed at  $850^\circ$  C.  $\times 3$  hours, and the maximum magnetic permeability and a coercive force were measured using a DC magnetization specific test device. Table 2 shows the observation results.

TABLE 2

| Sample No. | grain size number | Area ratio (%) of crystal grains having a GOS value of $0.5^\circ$ or more |                          |                       | Maximum magnetic permeability | Coercive force (A/m)         | Note |
|------------|-------------------|----------------------------------------------------------------------------|--------------------------|-----------------------|-------------------------------|------------------------------|------|
|            |                   | Vertical cross section                                                     | Horizontal cross section | magnetic permeability |                               |                              |      |
| 1          | 8.0               | 85                                                                         | 87                       | 19,600                | 39                            | Example of present invention |      |
| 2          | 9.0               | 62.5                                                                       | 40.2                     | 18,600                | 42                            | Comparative example          |      |

Table 2 shows the result in which Sample No. 1, which is the example of the present invention, had a smaller average crystal grain size number than Sample No. 2, which is a comparative example (had a larger crystal grain size than the comparative example). Regarding the area ratio of crystal grains having a GOS value of  $0.5^\circ$  or more, it was confirmed that the example of the present invention had a much larger value of the area ratio than the comparative example, and the difference between the horizontal cross section and the vertical cross section was small. Regarding the magnetic properties, Sample No. 1, which is the example of the present invention, had higher magnetic permeability and a lower coercive force than Sample No. 2, which is the comparative example. Accordingly, it was confirmed that the example of the present invention had better magnetic properties than the comparative example.

What is claimed is:

1. An Fe—Co-based alloy bar comprising 25 to 60% of Co, a total of one or more elements of V, Si, Mn, Al, Zr, B,

Ni, Ta, Nb, W, Ti, Mo, and Cr in a maximum mass % of 5.0%, and 95% or more of Fe and Co in mass %, wherein a diameter of a circular cross-sectional shape of the Fe—Co-based alloy bar is in a range of 5 mm to 20 mm,

an area ratio of crystal grains having a grain orientation spread (GOS) value of  $0.5^\circ$  or more exceeds 80%, and the difference between an area ratio of crystal grains having a GOS value of  $0.5^\circ$  or more observed in a cross section in a direction perpendicular to an axis of the bar and an area ratio of crystal grains having a GOS value of  $0.5^\circ$  or more observed in a cross section in an axial direction of the bar is within 10%, wherein the GOS value is measured by electron backscatter diffraction (SEM-EBSD) method.

2. The Fe—Co-based alloy bar according to claim 1, wherein an average crystal grain size number as measured according to JISG 0551 is 6.0 or more and 8.5 or less.

\* \* \* \* \*